



US007923423B2

(12) **United States Patent**  
**Walker et al.**

(10) **Patent No.:** **US 7,923,423 B2**  
(b5) **Date of Patent:** **Apr. 12, 2011**

(54) **COMPOSITIONS FOR PROCESSING OF SEMICONDUCTOR SUBSTRATES**

(75) Inventors: **Elizabeth Walker**, Nazareth, PA (US); **Shahri Naghshineh**, Allentown, PA (US); **Jeff Barnes**, Bath, PA (US); **Ewa Oldak**, Bethlehem, PA (US)

(73) Assignee: **Advanced Technology Materials, Inc.**, Danbury, CT (US)

(\*) Notice: Subject to any disclaimer, the term of this patent is extended or adjusted under 35 U.S.C. 154(b) by 400 days.

(21) Appl. No.: **11/046,262**

(22) Filed: **Jan. 27, 2005**

(65) **Prior Publication Data**

US 2006/0166847 A1 Jul. 27, 2006

(51) **Int. Cl.**  
**C11D 7/50** (2006.01)

(52) **U.S. Cl.** ..... **510/175**; 510/176; 134/1.3

(58) **Field of Classification Search** ..... **510/175**, 510/176; 134/1.3

See application file for complete search history.

(56) **References Cited**

U.S. PATENT DOCUMENTS

|               |         |                           |
|---------------|---------|---------------------------|
| 5,174,816 A   | 12/1992 | Aoyama et al.             |
| 5,308,745 A   | 5/1994  | Schwartzkopf              |
| 5,334,332 A   | 8/1994  | Lee                       |
| 5,466,389 A   | 11/1995 | Ilardi et al.             |
| 5,489,557 A   | 2/1996  | Jolley                    |
| 5,498,293 A * | 3/1996  | Ilardi et al. .... 134/3  |
| 5,563,119 A   | 10/1996 | Ward                      |
| 5,567,574 A   | 10/1996 | Hasemi et al.             |
| 5,571,447 A   | 11/1996 | Ward et al.               |
| 5,597,420 A   | 1/1997  | Ward                      |
| 5,612,304 A * | 3/1997  | Honda et al. .... 510/176 |

|                |         |                                |
|----------------|---------|--------------------------------|
| 5,759,973 A *  | 6/1998  | Honda et al. .... 510/176      |
| 5,795,702 A    | 8/1998  | Tanabe et al.                  |
| 5,855,811 A    | 1/1999  | Grieger et al.                 |
| 5,863,344 A    | 1/1999  | Nam                            |
| 5,885,362 A *  | 3/1999  | Morinaga et al. .... 134/2     |
| 5,962,384 A    | 10/1999 | Cooper et al.                  |
| 5,981,454 A    | 11/1999 | Small                          |
| 5,988,186 A    | 11/1999 | Ward et al.                    |
| 5,989,353 A *  | 11/1999 | Skee et al. .... 134/2         |
| 5,997,658 A    | 12/1999 | Peters et al.                  |
| 6,030,932 A *  | 2/2000  | Leon et al. .... 510/175       |
| 6,143,705 A    | 11/2000 | Kakizawa et al.                |
| 6,194,366 B1 * | 2/2001  | Naghshineh et al. .... 510/175 |
| 6,228,823 B1   | 5/2001  | Morinaga et al.                |
| 6,395,693 B1   | 5/2002  | Wang                           |
| 6,410,494 B2   | 6/2002  | Kakizawa et al.                |
| 6,413,923 B2   | 7/2002  | Honda et al.                   |
| 6,440,326 B1   | 8/2002  | Maruyama et al.                |

(Continued)

FOREIGN PATENT DOCUMENTS

EP 0773480 A1 5/1997

(Continued)

Primary Examiner — Gregory E Webb

(74) Attorney, Agent, or Firm — Tristan A. Fuirer; Moore & Van Allen, PLLC; Chih-Sheng Lin

(57) **ABSTRACT**

Compositions useful in semiconductor manufacturing for surface preparation and/or cleaning of wafer substrates such as semiconductor device precursor structures. The compositions can be employed for processing of wafers that have, or are intended to be further processed to include, copper metallization, e.g., in operations such as surface preparation, pre-plating cleaning, post-etching cleaning, and post-chemical mechanical polishing cleaning of semiconductor wafers. The compositions contain (i) alkanolamine, (ii) quaternary ammonium hydroxide and (iii) a complexing agent, and are storage-stable, as well as non-darkening and degradation-resistant in exposure to oxygen.

**35 Claims, 14 Drawing Sheets**



# US 7,923,423 B2

Page 2

---

## U.S. PATENT DOCUMENTS

|              |      |         |                      |
|--------------|------|---------|----------------------|
| 6,492,308    | B1   | 12/2002 | Naghshineh et al.    |
| 6,514,434    | B1   | 2/2003  | He et al.            |
| 6,514,921    | B1   | 2/2003  | Kakizawa et al.      |
| 6,585,825    | B1 * | 7/2003  | Skee .....           |
| 6,599,370    | B2   | 7/2003  | Skee .....           |
| 6,627,587    | B2   | 9/2003  | Naghshineh et al.    |
| 6,638,694    | B2   | 10/2003 | Ikemoto et al.       |
| 6,723,691    | B2   | 4/2004  | Naghshineh et al.    |
| 6,797,682    | B2   | 9/2004  | Hara et al.          |
| 6,992,050    | B2   | 1/2006  | Koita et al.         |
| 7,375,066    | B2   | 5/2008  | Kakizawa et al.      |
| 7,723,280    | B2   | 5/2010  | Brainard et al.      |
| 2001/0001785 | A1 * | 5/2001  | Honda et al. ....    |
| 2002/0128164 | A1   | 9/2002  | Hara et al.          |
| 2002/0132745 | A1   | 9/2002  | Honda et al.         |
| 2003/0130147 | A1 * | 7/2003  | Koito et al. ....    |
| 2003/0145908 | A1 * | 8/2003  | Fukumura et al. .... |
| 2003/0181342 | A1   | 9/2003  | Seijo et al.         |
| 2003/0235996 | A1 * | 12/2003 | Leon et al. ....     |
| 2004/0106531 | A1 * | 6/2004  | Kanno et al. ....    |
| 2004/0137379 | A1 * | 7/2004  | Ikemoto .....        |
| 2004/0137736 | A1   | 7/2004  | Daviot et al.        |
| 2004/0180300 | A1   | 9/2004  | Minsek et al.        |

|              |      |         |                       |
|--------------|------|---------|-----------------------|
| 2004/0220065 | A1   | 11/2004 | Hsu                   |
| 2004/0224866 | A1 * | 11/2004 | Matsunaga et al. .... |
| 2005/0100621 | A1 * | 5/2005  | Popp et al. ....      |
| 2005/0106492 | A1   | 5/2005  | Yokoi et al.          |
| 2005/0181961 | A1 * | 8/2005  | Misra et al. ....     |
| 2005/0197265 | A1   | 9/2005  | Rath et al.           |
| 2005/0205835 | A1 * | 9/2005  | Tamboli et al. ....   |
| 2005/0287480 | A1 * | 12/2005 | Takashima .....       |
| 2006/0016785 | A1   | 1/2006  | Egbe et al.           |
| 2006/0073997 | A1   | 4/2006  | Leonte et al.         |
| 2006/0148666 | A1   | 7/2006  | Peters et al.         |

## FOREIGN PATENT DOCUMENTS

|    |             |         |
|----|-------------|---------|
| JP | 63274149 A  | 11/1988 |
| JP | 07-201794 A | 8/1995  |
| JP | 07-247498 A | 9/1995  |
| JP | 08-202052 A | 8/1996  |
| JP | 11-271985 A | 10/1999 |
| WO | 9408276     | 4/1994  |
| WO | WO94/08276  | 4/1994  |
| WO | 9816330     | 4/1998  |
| WO | 9960448     | 11/1999 |

\* cited by examiner

**FIG. 1****FIG. 2**



**FIG. 3**



**FIG 4**



**FIG. 5**



**FIG. 6**

**FIG 7****FIG. 8**

**FIG. 9**

**FIG. 10**

**FIG. 11****FIG. 12**

**FIG. 13****FIG. 14**

**FIG. 15****FIG. 16**



**FIG. 17**



**FIG. 18**



**FIG. 19**



**FIG. 20**

**FIG. 21****FIG. 22**



**FIG. 23**



**FIG. 24**



**FIG. 25**

## 1

## COMPOSITIONS FOR PROCESSING OF SEMICONDUCTOR SUBSTRATES

## FIELD OF THE INVENTION

The present invention relates to compositions for processing of semiconductor substrates, including compositions useful for surface preparation, pre-plating cleaning, post-etch cleaning, and post-chemical mechanical polishing cleaning of semiconductor wafers.

## DESCRIPTION OF THE RELATED ART

Semiconductor wafers are used to form integrated circuits. The semiconductor wafer includes a substrate, such as silicon, into which regions are patterned for deposition of different materials having insulative, conductive or semi-conductive properties.

In order to obtain the correct patterning, excess material used in forming the layers on the substrate must be removed. Further, to fabricate functional and reliable circuitry, it is important to have a flat or planar semiconductor wafer surface. Thus, it is necessary to remove and/or polish certain surfaces of a semiconductor wafer.

Chemical Mechanical Polishing or Planarization ("CMP") is a process in which material is removed from a surface of a semiconductor wafer, and the surface is polished (planarized) by coupling a physical process such as abrasion with a chemical process such as oxidation or chelation. In its most rudimentary form, CMP involves applying slurry, a solution of an abrasive and an active chemistry, to a polishing pad that buffs the surface of a semiconductor wafer to achieve the removal, planarization, and polishing process. It is not desirable for the removal or polishing process to be comprised of purely physical or purely chemical action, but rather the synergistic combination of both in order to achieve fast uniform removal. In the fabrication of integrated circuits, the CMP slurry should also be able to preferentially remove films that comprise complex layers of metals and other materials so that highly planar surfaces can be produced for subsequent photolithography, or patterning, etching and thin-film processing.

Recently, copper has been increasingly used for metal interconnects in integrated circuits. In the copper damascene process commonly used for metallization of circuitry in semiconductor fabrication, the layers that must be removed and planarized include copper layers having a thickness of about 1-1.5  $\mu\text{m}$  and copper seed layers having a thickness of about 0.05-0.15  $\mu\text{m}$ . These copper layers are separated from the dielectric material surface by a layer of barrier material, typically about 50-300  $\text{\AA}$  thick, which prevents diffusion of copper into the oxide dielectric material. The key to obtaining good uniformity across the wafer surface after polishing is to use a CMP slurry that has the correct removal selectivities for each material.

The foregoing processing operations, involving wafer substrate surface preparation, deposition, plating, etching and chemical mechanical polishing, variously require cleaning operations to ensure that the semiconductor product is free of contaminants that would otherwise deleteriously affect the function of the product, or even render it useless for its intended function.

One particular issue in this respect is the residues that are left on the semiconductor device substrate following CMP processing. Such residues include CMP material and corrosion inhibitor compounds such as benzotriazole (BTA). If not removed, these residues can cause damage to copper lines or severely roughen the copper metallization, as well as cause

## 2

poor adhesion of post-CMP applied layers on the device substrate. Severe roughening of copper metallization is particularly problematic, since overly rough copper can cause poor electrical performance of the product semiconductor device.

The following patents illustrate various formulations for cleaning of semiconductor substrates. One type of cleaning formulation that is employed with copper metallized substrates is described in U.S. Pat. Nos. 6,194,366 and 6,492,308 and contains tetramethylammonium hydroxide (TMAH), monoethanolamine (MEA), copper corrosion inhibitor and water. The disadvantages of such formulations include their susceptibility to degradation when exposed to oxygen, which in turn results in darkening of the color of the formulation, with the result that sensors associated with semiconductor process tools yield erroneous outputs that may compromise the function and reliability of the tool. Additionally, such degradation involves loss of cleaning ability, which may be sufficiently extensive in the case of prolonged oxygen exposure that the cleaning formulation has no significant efficacy.

For these reasons, cleaning formulations of the type disclosed in U.S. Pat. Nos. 6,194,366 and 6,492,308 must be maintained under nitrogen blanket, or otherwise secured against oxygen exposure.

The microelectronics industry therefore continues to seek improvement in cleaning formulations for copper-metallized substrates, and in compositions for processing of semiconductor device structures, including compositions variously useful for surface preparation, pre-plating cleaning, post-etching cleaning, and post-chemical mechanical polishing cleaning of semiconductor wafers.

## SUMMARY OF THE INVENTION

The present invention relates to compositions for processing of semiconductor substrates, including compositions variously useful for surface preparation, pre-plating cleaning, post-etch cleaning, and post-chemical mechanical polishing of semiconductor wafers.

In one aspect, the invention relates to a composition including (i) alkanolamine, (ii) quaternary ammonium hydroxide and (iii) a complexing agent, wherein the complexing agent includes at least one component selected from the group consisting of acetic acid, acetone oxime, alanine, 5-aminotetrazole, arginine, asparagine, aspartic acid, benzoic acid, betaine, dimethyl glyoxime, fumaric acid, glutamic acid, glutamine, glutaric acid, glycerol, glycine, glycolic acid, glyoxylic acid, histidine, imidazole, iminodiacetic acid, isophthalic acid, itaconic acid, lactic acid, leucine, lysine, maleic acid, malic acid, malonic acid, 2-mercaptopbenzimidazole, oxalic acid, 2,4-pentanedione, phenylacetic acid, phenylalanine, phthalic acid, proline, pyromellitic acid, quinic acid, serine, sorbitol, succinic acid, terephthalic acid, 1,2,4-triazole, trimellitic acid, trimesic acid, tyrosine, valine, xylitol, and derivatives of the foregoing amino acids, with the provision that the complexing agent does not include citric acid.

In another aspect, the invention relates to a method of processing a semiconductor substrate to remove undesired material therefrom or to prepare a surface of said semiconductor substrate for subsequent treatment, such method including contacting the semiconductor substrate with an effective amount of a composition comprising (i) alkanolamine, (ii) quaternary ammonium hydroxide and (iii) a complexing agent, wherein the complexing agent includes at least one component selected from the group consisting of acetic acid, acetone oxime, alanine, 5-aminotetrazole, arginine, asparagine, aspartic acid, benzoic acid, betaine, dimethyl gly-

oxime, fumaric acid, glutamic acid, glutamine, glutaric acid, glycerol, glycine, glycolic acid, glyoxylic acid, histidine, imidazole, iminodiacetic acid, isophthalic acid, itaconic acid, lactic acid, leucine, lysine, maleic acid, malic acid, malonic acid, 2-mercaptopbenzimidazole, oxalic acid, 2,4-pentanedione, phenylacetic acid, phenylalanine, phthalic acid, proline, pyromellitic acid, quinic acid, serine, sorbitol, succinic acid, terephthalic acid, trimellitic acid, 1,2,4-triazole, trimesic acid, tyrosine, valine, xylitol, and derivatives of the foregoing amino acids, with the provision that the complexing agent does not include citric acid.

Other aspects, features and embodiments of the invention will be more fully apparent from the ensuing disclosure and appended claims.

#### BRIEF DESCRIPTION OF THE DRAWINGS

FIG. 1 is a photomicrograph of a cobalt-plated semiconductor device structure that has been plated subsequent to surface preparation with an aqueous composition AV including TMAH, MEA and TEA, without a complexing agent.

FIG. 2 is a photomicrograph of a cobalt-plated semiconductor device structure that has been plated subsequent to surface preparation with an aqueous composition AW including TMAH, MEA, TEA, and lactic acid.

FIG. 3 is a photomicrograph of a cobalt-plated semiconductor device structure that has been plated subsequent to surface preparation with an aqueous composition AX including TMAH, MEA, TEA, and oxalic acid.

FIG. 4 is a photomicrograph of a cobalt-plated semiconductor device structure that has been plated subsequent to surface preparation with an aqueous composition AY including TMAH, MEA, TEA, and citric acid.

FIG. 5 is a photomicrograph of a cobalt-plated semiconductor device structure that has been plated subsequent to surface preparation with an aqueous composition AZ including TMAH, aminoethoxyethanol, dimethylaminoethoxyethanol, and lactic acid.

FIG. 6 is a photomicrograph of a cobalt-plated semiconductor device structure that has been plated subsequent to surface preparation with an aqueous composition BA including TMAH, aminoethoxyethanol, dimethylaminoethoxyethanol, and oxalic acid.

FIG. 7 is a photomicrograph of a cobalt-plated semiconductor device structure that has been plated subsequent to surface preparation with an aqueous composition BB including TMAH, aminoethoxyethanol, dimethylaminoethoxyethanol, and citric acid.

FIG. 8 is a graph of etch rate, in Angstroms per minute, for TMAH/MEA compositions P, AA, U, AQ, BT, and BU containing different complexing agents (gallic acid, lactic acid, glycine and succinic acid, respectively) on a copper substrate.

FIG. 9 is a graph of surface roughness, in nm, for various TMAH/MEA compositions, showing the relative magnitudes of the roughness associated with varying complexing agents, against an untreated copper surface having a roughness of 1.4 nm.

FIG. 10 is a graph of surface roughness, in nm, for various TMAH/MEA compositions, showing the relative magnitudes of the roughness associated with varying complexing agents, against an untreated copper surface having a roughness of 1.4 nm.

FIG. 11 is a photomicrograph at magnification of 40,000 $\times$  of a post-etch wafer showing residue in vias therein.

FIG. 12 is a photomicrograph of the post-etch wafer of FIG. 11, at a magnification of 80,000 $\times$ , showing the residue in the vias, in greater detail.

FIG. 13 is a photomicrograph at magnification of 40,000 $\times$  of the post-etch wafer shown in FIG. 11, after cleaning by spin/spray with a TMAH/MEA/lactic acid aqueous cleaning composition AA. The residue has been removed.

5 FIG. 14 is a photomicrograph of the post-etch wafer of FIG. 13, at a magnification of 80,000 $\times$ , showing the removal of the post-etch residue in the via, in greater detail.

FIG. 15 is a photomicrograph at magnification of 40,000 $\times$  of the post-etch wafer shown in FIG. 11, after cleaning by spin/spray with a TMAH/MEA/glycine aqueous cleaning composition U. The residue has been removed.

10 FIG. 16 is a photomicrograph of the post-etch wafer of FIG. 15, at a magnification of 80,000 $\times$ , showing the removal of the post-etch residue in the via, in greater detail.

15 FIG. 17 is a photomicrograph at magnification of 40,000 $\times$  of the post-etch wafer shown in FIG. 11, after cleaning by spin/spray with a TH/MEA/succinic acid aqueous cleaning composition AQ. The residue has been removed.

FIG. 18 is a photomicrograph of the post-etch wafer of FIG. 17, at a magnification of 80,000 $\times$ , showing the removal of the post-etch residue in the via, in greater detail.

20 FIG. 19 is a photomicrograph at magnification of 40,000 $\times$  of the post-etch wafer shown in FIG. 11, after cleaning by spin/spray with a TMAH/MEA/ascorbic acid aqueous cleaning composition CO. The residue has been removed.

25 FIG. 20 is a photomicrograph of the post-etch wafer of FIG. 19, at a magnification of 80,000 $\times$ , showing the post-etch residue remaining in the via, in greater detail.

FIG. 21 is a photomicrograph at magnification of 40,000 $\times$  30 of the post-etch wafer shown in FIG. 11, after immersion cleaning with a TMAH/MEA/lactic acid aqueous cleaning composition AA. The residue has been removed.

FIG. 22 is a photomicrograph of the post-etch wafer of FIG. 21, at a magnification of 80,000 $\times$ , showing the removal 35 of the post-etch residue in the via, in greater detail.

FIG. 23 is a photomicrograph at magnification of 40,000 $\times$  of the post-etch wafer shown in FIG. 11, after immersion cleaning with a TMAH/MEA/glycine aqueous cleaning composition U. The residue has been removed.

40 FIG. 24 is a photomicrograph at magnification of 40,000 $\times$  of the post-etch wafer shown in FIG. 11, after immersion cleaning with a TMAH/MEA/succinic acid aqueous cleaning composition AQ. The residue has been removed.

FIG. 25 is a photomicrograph of the post-etch wafer of FIG. 24, at a magnification of 80,000 $\times$ , showing the removal 45 of the post-etch residue in the via, in greater detail.

#### DETAILED DESCRIPTION OF THE INVENTION, AND PREFERRED EMBODIMENTS THEREOF

The present invention relates to compositions that are variously useful in semiconductor manufacturing, e.g., for processing of wafer articles that have or are intended to be further processed to have copper metallization, in operations such as 50 surface preparation, pre-plating cleaning, post-etching cleaning, and post-chemical mechanical polishing cleaning of semiconductor wafers.

The compositions of the invention are aqueous compositions including (i) alkanolamine, (ii) quaternary ammonium hydroxide and (iii) a complexing agent, which are present in the composition in relative amounts imparting to the composition an effectiveness for the intended surface preparation and/or cleaning for which the composition is used. For example, the composition may include 0.001-90 wt. % 55 alkanolamine, 0.005-50 wt. % quaternary ammonium hydroxide, 0.001-20 wt. % complexing agent, and the balance water. The composition in a preferred embodiment is formulated so

that the alkalinity of the solution is greater than 0.004 miliequivalents of base per gram of solution.

In accordance with the invention, the complexing agent in such compositions includes at least one component selected from the group consisting of acetic acid, acetone oxime, alanine, 5-aminotetrazole, arginine, asparagine, aspartic acid, benzoic acid, betaine, dimethyl glyoxime, fumaric acid, glutamic acid, glutamine, glutaric acid, glycerol, glycine, glycolic acid, glyoxylic acid, histidine, imidazole, iminodiacetic acid, isophthalic acid, itaconic acid, lactic acid, leucine, lysine, maleic acid, malic acid, malonic acid, 2-mercaptopbenzimidazole, oxalic acid, 2,4-pentanedione, phenylacetic acid, phenylalanine, phthalic acid, proline, pyromellitic acid, quinic acid, serine, sorbitol, succinic acid, terephthalic acid, 1,2,4-triazole, trimellitic acid, trimesic acid, tyrosine, valine, xylitol, and derivatives of the foregoing amino acids, provided, however, that the complexing agent does not include citric acid.

In a specific aspect, the complexing agent may be formulated so that it additionally does not contain gallic acid or ascorbic acid.

In various embodiments, the compositions of the invention may be formulated so as to alternatively comprise, consist or consist essentially of, specific components identified herein as ingredients of such compositions.

The complexing agent serves to facilitate cleaning and surface preparation of substrates, e.g., semiconductor substrates requiring cleaning and/or surface preparation.

The compositions of the invention are air-stable in character (i.e., oxidation-resistant). As a result, the compositions of the invention can be utilized in the semiconductor fab without the necessity of nitrogen blanketing, or vacuum or other inert environments to maintain their stability and color.

Specific compositions within the broad scope of the invention variously include: compositions having utility for post-chemical mechanical planarization (PCMP) cleaning of semiconductor substrates; compositions having utility for surface preparation of semiconductor substrates for metals plating; and compositions having utility for cleaning of semiconductor substrates after etch processing thereof.

In various applications, the compositions of the invention may be utilized in a highly concentrated form, which is taken here to refer to compositions containing less than 20% by weight water, based on the total weight of the composition, preferably an amount of water in a range of from 2 to 20 wt. % water, more preferably in a range of from 3 to 10 wt. % water, and most preferably in a range of from 3 to 8 wt. % water. Such concentrated compositions are particularly useful for surface preparation of semiconductor wafers and for very difficult to remove photo etch and photoresist residues. It will be appreciated that in general cleaning applications, it is common practice to make highly concentrated forms to be used at extreme dilutions. The formulations in the examples can be made more concentrated for higher dilution at the point of use.

In other applications, the compositions of the invention may be utilized in a highly dilute form, which is taken here as referring to compositions containing at least 95% water, preferably an amount of water in a range of from 95 to 99.999 wt. % water, more preferably in a range of from 97 to 99.99 wt. % water, and most preferably in a range of from 98 to 99.9 wt. % water. Such dilute compositions are particularly useful for PCMP processing of semiconductor device structures, for removing CMP residue from the surface of the structure, or for preparing surfaces for subsequent plating operations as well as for cleaning of etch residues from the surface of semiconductor substrates after etch processing thereof.

The compositions of the invention include alkanolamine, which can be of any suitable type, and is typically present in an amount of from about 0.001% to about 90% by weight, based on the weight of the composition. Illustrative alkanolamines that may be useful in specific compositions include, without limitation, aminoethylethanolamine, N-methylaminoethanol, aminoethoxyethanol, dimethylaminoethoxyethanol, diethanolamine, N-methyldiethanolamine, monoethanolamine, triethanolamine, C<sub>1</sub>-C<sub>8</sub> alkanolamines, and combinations thereof.

The concentration of the alkanolamine in highly concentrated compositions of the invention may be in a range of from about 2 to about 90 wt %, based on the weight of the composition, more preferably in a range of from about 4 to about 45 wt %, and most preferably in a range of from about 6 to about 35 wt %, on the same total weight basis.

The concentration of the alkanolamine in highly dilute compositions of the invention may be in a range of from about 0.001 to about 6 wt %, based on the weight of the composition, more preferably in a range of from about 0.01 to about 2.5 wt %, and most preferably in a range of from about 0.06 to about 2 wt %, on the same total weight basis.

Compositions in accordance with the invention also include quaternary ammonium hydroxide, typically present in an amount of from about 0.005% to about 40% by weight, based on the weight of the composition. The quaternary ammonium hydroxide can be of any suitable type. Illustrative quaternary ammonium hydroxides that may be useful in specific compositions include, without limitation, choline, tetrabutylammoniumhydroxide, tetraethylammonium hydroxide, tetramethylammonium hydroxide, and tetrapropylammoniumhydroxide, and combinations thereof.

The concentration of the quaternary ammonium hydroxide in highly concentrated compositions of the invention may be in a range of from about 0.01 to about 40 wt %, based on the weight of the composition, more preferably in a range of from about 0.1 to about 20 wt %, and most preferably in a range of from about 0.5 to about 5 wt %, on the same total weight basis.

The concentration of the quaternary ammonium hydroxide in highly dilute compositions of the invention may be in a range of from about 0.00001 to about 2.5 wt %, based on the weight of the composition, more preferably in a range of from about 0.0005 to about 1.5 wt %, and most preferably in a range of from about 0.005 to about 0.5 wt %, on the same total weight basis.

The concentration of the complexing agent may be any suitable concentration at which the complexing agent is effective to provide enhancement of the surface preparation and/or cleaning for which the composition containing same is intended to be used. Typically the concentration of the complexing agent is in a range of from about 0.001 wt. % to about 20 wt. %, based on the total weight of the composition (complexing agent, alkanolamine, quaternary ammonium hydroxide, and water).

The concentration of the complexing agent in highly concentrated compositions of the invention may be in a range of from about 0.01 to about 20 wt %, based on the weight of the composition, more preferably in a range of from about 0.1 to about 12 wt %, and most preferably in a range of from about 0.5 to about 5 wt %, on the same total weight basis.

The concentration of the complexing agent in highly dilute compositions of the invention may be in a range of from about 0.00001 to about 2.5 wt %, based on the weight of the composition, more preferably in a range of from about 0.0005 to about 1.5 wt %, and most preferably in a range of from about 0.005 to about 0.5 wt %, on the same total weight basis. The compositions of the invention include water in an appropriate amount for the intended end use of the composition, with

surface preparation compositions generally containing larger amounts of water than is employed in compositions intended for removal of residues, particulates and other detritus from the substrate being cleaned. The water is preferably deionized water, and may be produced by distillation, filtration and/or other purification operations, to provide an aqueous medium for the composition, having appropriate character.

The pH of the compositions may be varied to produce a composition optimized for the intended end use. In general, the pH will be basic, e.g., greater than 9, with compositions preferably having pH greater than 9.5 and more preferably greater than 10 being usefully employed for surface preparation and/or cleaning in specific embodiments of the invention.

The compositions of the invention may also be formulated to have specific alkalinity characteristics, e.g., a concentrated chemical may have an alkalinity in a range of from about 0.9 to about 3.5 milliequivalents base per gram of solution.

Compositions of the invention are stable in character, and do not degrade in the manner of the TMAH/MEA-based formulations of the prior art. Thus, the compositions are storage stable, without loss of efficacy, and resistant to oxygen-mediated degradation, so that they may be used in ambient air environments, without darkening and loss of effectiveness. For these reasons, the compositions of the present invention represent a striking improvement over the TMAH/MEA-based formulations of the prior art, and retain a clear and transparent character even after prolonged exposure to oxygen or oxygen-containing gases such as air.

In addition to not changing color over time or upon exposure to oxygen, the compositions of the invention exhibit low copper roughening, good PCMP cleaning, good BTA removal, and good post etch residue removal characteristics.

The cleaning solution of the invention does not require a surfactant in the formulation, however this does not preclude the use of surfactants in cleaning solutions of the invention, in specific applications where such agents may be beneficial.

In one specific embodiment, the invention discloses relates to compositions having utility for post etch removal of residue from semiconductor substrates; these compositions include alkanolamine, quaternary ammonium hydroxide, complexing agent, and the balance water, in the following composition:

---

|                                                                                                                |            |
|----------------------------------------------------------------------------------------------------------------|------------|
| alkanolamine, e.g. monoethanolamine                                                                            | 9 wt. %;   |
| quaternary ammonium hydroxide, e.g. tetramethyl ammonium hydroxide                                             | 5 wt. %;   |
| complexing agent, e.g. lactic acid                                                                             | 1.9 wt. %; |
| and the balance water, wherein the weight percentages of all components of the composition total to 100 wt. %. |            |

---

In another specific embodiment, the invention relates to compositions having utility for post CMP removal of residue from surface preparation of semiconductor substrates; these compositions include alkanolamine, quaternary ammonium hydroxide, complexing agent, and the balance water, in the following composition:

---

|                                                                                                                |              |
|----------------------------------------------------------------------------------------------------------------|--------------|
| alkanolamine, e.g. monoethanolamine                                                                            | 0.3 wt. %;   |
| quaternary ammonium hydroxide, e.g. tetramethyl ammonium hydroxide                                             | 0.166 wt. %; |
| complexing agent, e.g. terephthalic acid                                                                       | 0.004 wt. %; |
| and the balance water, wherein the weight percentages of all components of the composition total to 100 wt. %. |              |

---

In a specific embodiment, useful for the cleaning of semiconductor substrates to remove residues therefrom, the composition may contain 9 wt. % alkanolamine, e.g., monoethanolamine, 5 wt. % quaternary ammonium hydroxide, e.g., tetramethylammonium hydroxide, and a complexing agent such as lactic acid, in an amount of 1.85 wt. %, or glycine in an amount of 2.4 wt. %, or succinic acid in an amount of 2.4 wt. %, with the balance of the composition being water.

In another specific embodiment, useful for surface treatment of a semiconductor substrate for subsequent cobalt plating, the composition may contain 5 wt. % tetramethylammonium hydroxide, 18.5 wt. % dimethylaminoethoxyethanol, 1.9 wt. % oxalic acid dihydrate, and the balance water.

The compositions of the invention may be prepared as a concentrate of the alkanolamine, quaternary ammonium hydroxide, and complexing agent components, which are storable and transportable in such form, for subsequent addition of water at the point of use. In general cleaning applications, it is common practice to make highly concentrated forms to be used at extreme dilutions. The formulations in the examples can be made more concentrated for higher dilution at the point of use. For such purpose, the concentrate may be dissolved in water at up to 500:1 dilutions, e.g., at dilutions of 20:1, 40:1, or 100:1 of the diluent water to the concentrate (volumetric dilution basis).

In some instances, it may be desirable to use the concentrate in a neat, i.e., non-diluted form, to provide enhanced cleaning or surface preparation action. The nature and extent of the dilution can be widely varied to good effect, within the broad scope of the invention.

The following Examples are merely illustrative of the invention and are not intended to be limiting.

#### COMPOSITIONS FOR EXAMPLES

The compositions used in the ensuing examples are identified below (all percentages by weight, based on the total weight of the composition including water).

Composition A: 9% monoethanolamine, 5% tetramethyl ammonium hydroxide, 1.2% acetic acid, balance water

Composition B: 9% monoethanolamine, 5% tetramethyl ammonium hydroxide, 1.5% acetone oxime, balance water

Composition C: 9% monoethanolamine, 5% tetramethyl ammonium hydroxide, 1.8% alanine, balance water

Composition D: 9% monoethanolamine, 5% tetramethyl ammonium hydroxide, 1.8% 5-aminotetrazole, balance water

Composition E: 9% monoethanolamine, 5% tetramethyl ammonium hydroxide, 2.7% asparagine, balance water

Composition F: 9% monoethanolamine, 5% tetramethyl ammonium hydroxide, 3.6% arginine, balance water

Composition G: 9% monoethanolamine, 5% tetramethyl ammonium hydroxide, 2.7% aspartic acid, balance water

Composition H: 9% monoethanolamine, 5% tetramethyl ammonium hydroxide, 2.4% betaine, balance water

Composition I: 9% monoethanolamine, 5% tetramethyl ammonium hydroxide, 4.0% citric acid, balance water

Composition J: 9% monoethanolamine, 5% tetramethyl ammonium hydroxide, 2.7% cyanuric acid, balance water

Composition K: 9% monoethanolamine, 5% tetramethyl ammonium hydroxide, 2.5% cysteine, balance water

Composition L: 9% monoethanolamine, 5% tetramethyl ammonium hydroxide, 2.4% dimethyl glyoxime, balance water

Composition M: 9% monoethanolamine, 5% tetramethyl ammonium hydroxide, 1.2% ethylene diamine, balance water

Composition N: 9% monoethanolamine, 5% tetramethyl ammonium hydroxide, 2.4% fumaric acid, balance water  
 Composition O: 9% monoethanolamine, 5% tetramethyl ammonium hydroxide, 4.3% glucarate, balance water  
 Composition P: 9% monoethanolamine, 5% tetramethyl ammonium hydroxide, 3.5% gallic acid, balance water  
 Composition Q: 9% monoethanolamine, 5% tetramethyl ammonium hydroxide, 3.0% glutamic acid, balance water  
 Composition R: 9% monoethanolamine, 5% tetramethyl ammonium hydroxide, 3.0% glutamine, balance water  
 Composition S: 9% monoethanolamine, 5% tetramethyl ammonium hydroxide, 2.7% glutaric acid, balance water  
 Composition T: 9% monoethanolamine, 5% tetramethyl ammonium hydroxide, 1.9% glycerol, balance water  
 Composition U: 9% monoethanolamine, 5% tetramethyl ammonium hydroxide, 1.6% glycine, balance water  
 Composition V: 9% monoethanolamine, 5% tetramethyl ammonium hydroxide, 1.6% glycolic acid, balance water  
 Composition W: 9% monoethanolamine, 5% tetramethyl ammonium hydroxide, 3.2% histidine, balance water  
 Composition X: 9% monoethanolamine, 5% tetramethyl ammonium hydroxide, 1.4% imidazole, balance water  
 Composition Y: 9% monoethanolamine, 5% tetramethyl ammonium hydroxide, 2.7% iminodiacetic acid, balance water  
 Composition Z: 9% monoethanolamine, 5% tetramethyl ammonium hydroxide, 2.7% itaconic acid, balance water  
 Composition AA: 9% monoethanolamine, 5% tetramethyl ammonium hydroxide, 1.9% lactic acid, balance water  
 Composition AB: 9% monoethanolamine, 5% tetramethyl ammonium hydroxide, 2.7% leucine, balance water  
 Composition AC: 9% monoethanolamine, 5% tetramethyl ammonium hydroxide, 3.0% lysine, balance water  
 Composition AD: 9% monoethanolamine, 5% tetramethyl ammonium hydroxide, 2.4% maleic acid, balance water  
 Composition AE: 9% monoethanolamine, 5% tetramethyl ammonium hydroxide, 2.8% malic acid, balance water  
 Composition AF: 9% monoethanolamine, 5% tetramethyl ammonium hydroxide, 2.2% malonic acid, balance water  
 Composition AG: 9% monoethanolamine, 5% tetramethyl ammonium hydroxide, 3.1% 2-mercaptopbenzimidazole, balance water  
 Composition AH: 9% monoethanolamine, 5% tetramethyl ammonium hydroxide, 4.2% mucic acid, balance water  
 Composition AI: 9% monoethanolamine, 5% tetramethyl ammonium hydroxide, 1.9% oxalic acid, balance water  
 Composition AJ: 9% monoethanolamine, 5% tetramethyl ammonium hydroxide, 2.1% 2,4-pentanedione, balance water  
 Composition AK: 9% monoethanolamine, 5% tetramethyl ammonium hydroxide, 3.4% phenylalanine, balance water  
 Composition AM: 9% monoethanolamine, 5% tetramethyl ammonium hydroxide, 3.7% proline, balance water  
 Composition AN: 9% monoethanolamine, 5% tetramethyl ammonium hydroxide, 4.0% quinic acid, balance water  
 Composition AO: 9% monoethanolamine, 5% tetramethyl ammonium hydroxide, 2.2% serine, balance water  
 Composition AP: 9% monoethanolamine, 5% tetramethyl ammonium hydroxide, 3.8% sorbitol, balance water  
 Composition AQ: 9% monoethanolamine, 5% tetramethyl ammonium hydroxide, 2.4% succinic acid, balance water  
 Composition AR: 9% monoethanolamine, 5% tetramethyl ammonium hydroxide, 3.1% tartaric acid, balance water  
 Composition AS: 9% monoethanolamine, 5% tetramethyl ammonium hydroxide, 3.7% tyrosine, balance water  
 Composition AT: 9% monoethanolamine, 5% tetramethyl ammonium hydroxide, 2.4% valine, balance water

Composition AU: 9% monoethanolamine, 5% tetramethyl ammonium hydroxide, 3.1% xylitol, balance water  
 Composition AV: 21% triethanolamine, 1% monoethanolamine, 0.5% tetramethylammonium hydroxide, balance water  
 5 Composition AW: 21% triethanolamine, 1% monoethanolamine, 0.5% tetramethylammonium hydroxide, 1.9% lactic acid, balance water  
 Composition AX: 21% triethanolamine, 1% monoethanolamine, 0.5% tetramethylammonium hydroxide, 1.9% oxalic acid, balance water  
 Composition AY: 21% triethanolamine, 1% monoethanolamine, 0.5% tetramethylammonium hydroxide, 2.0% citric acid, balance water  
 10 Composition AZ: 18.7% dimethylaminoethoxyethanol, 0.9% aminoethoxyethanol, 0.5% tetramethylammonium hydroxide, 1.9% lactic acid, balance water  
 Composition BA: 18.7% dimethylaminoethoxyethanol, 0.9% aminoethoxyethanol, 0.5% tetramethylammonium hydroxide, 1.9% oxalic acid, balance water  
 15 Composition BB: 18.7% dimethylaminoethoxyethanol, 0.9% aminoethoxyethanol, 0.5% tetramethylammonium hydroxide, 2.0% citric acid, balance water  
 Composition BC: 21% triethanolamine, 1% monoethanolamine, 5% tetramethylammonium hydroxide, 1.9% lactic acid, balance water  
 20 Composition BD: 21% triethanolamine, 1% monoethanolamine, 5% tetramethylammonium hydroxide, 0.9% lactic acid, balance water  
 Composition BE: 10% triethanolamine, 1% monoethanolamine, 5% tetramethylammonium hydroxide, 1.9% lactic acid, balance water  
 25 Composition BF: 1% triethanolamine, 1% monoethanolamine, 5% tetramethylammonium hydroxide, 1.9% lactic acid, balance water  
 Composition BG: 21% triethanolamine, 1% monoethanolamine, 2.5% tetramethylammonium hydroxide, 1.9% lactic acid, balance water  
 30 Composition BH: 21% triethanolamine, 1% monoethanolamine, 5% tetramethylammonium hydroxide, 2.4% succinic acid, balance water  
 Composition BI: 21% triethanolamine, 1% monoethanolamine, 5% tetramethylammonium hydroxide, 2.2% malonic acid, balance water  
 35 Composition BJ: 21% triethanolamine, 0.9% 1-amino-2-propanol, 5% tetramethylammonium hydroxide, 1.9% lactic acid, balance water  
 Composition BK: 21% triethanolamine, 0.9% 2-amino-1-butanol, 5% tetramethylammonium hydroxide, 1.9% lactic acid, balance water  
 40 Composition BL: 21% triethanolamine, 0.9% 2-amino-2-methyl-1-propanol, 5% tetramethylammonium hydroxide, 1.9% lactic acid, balance water  
 Composition BM: 21% triethanolamine, 1% monoethanolamine, 5% tetramethylammonium hydroxide, 3.4% phthalic acid, balance water  
 45 Composition BN: 21% triethanolamine, 1% monoethanolamine, 5% tetramethylammonium hydroxide, 3.4% terephthalic acid, balance water  
 Composition BO: 18.7% dimethylaminoethoxyethanol, 1% monoethanolamine, 5% tetramethylammonium hydroxide, 1.9% lactic acid, balance water  
 50 Composition BP: 10.6% 2-methylaminoethanol, 1% monoethanolamine, 5% tetramethylammonium hydroxide, 1.9% lactic acid, balance water  
 55 Composition BR: 10.6% 2-methylaminoethanol, 1% monoethanolamine, 5% tetramethylammonium hydroxide, 1.9% lactic acid, balance water  
 Composition BS: 10.6% 2-methylaminoethanol, 1% monoethanolamine, 5% tetramethylammonium hydroxide, 1.9% lactic acid, balance water  
 60 Composition BT: 10.6% 2-methylaminoethanol, 1% monoethanolamine, 5% tetramethylammonium hydroxide, 1.9% lactic acid, balance water  
 Composition BU: 10.6% 2-methylaminoethanol, 1% monoethanolamine, 5% tetramethylammonium hydroxide, 1.9% lactic acid, balance water  
 65 Composition BV: 10.6% 2-methylaminoethanol, 1% monoethanolamine, 5% tetramethylammonium hydroxide, 1.9% lactic acid, balance water

## 11

Composition BQ: 18.7% dimethylaminoethoxyethanol, 0.9% aminoethoxyethanol, 5% tetramethylammonium hydroxide, 1.9% lactic acid, balance water.

Composition BR: 18.7% dimethylaminoethoxyethanol, 0.9% aminoethoxyethanol, 5% tetramethylammonium hydroxide, 3.4% terephthalic acid, balance water.

Composition BS: 18.7% dimethylaminoethoxyethanol, 0.9% aminoethoxyethanol, 5% tetramethylammonium hydroxide, 3.4% terephthalic acid, balance water.

Composition BT: 9% monoethanolamine, 5% tetramethyl ammonium hydroxide, 1.9% lactic acid, 0.5% 2-mercaptopbenzimidazole, balance water

Composition BU: 9% monoethanolamine, 5% tetramethyl ammonium hydroxide, 0.5% 2-mercaptopbenzimidazole, balance water

Composition CB: 0.3 wt % monoethanolamine, 0.166 wt % tetramethylammonium hydroxide, 0.003 wt % phenylacetic acid, balance water

Composition CC: 0.3 wt % monoethanolamine, 0.166 wt % tetramethylammonium hydroxide, 0.003 wt % acetic acid, balance water

Composition CD: 0.3 wt % monoethanolamine, 0.166 wt % tetramethylammonium hydroxide, 0.003 wt % benzoic acid, balance water

Composition CE: 0.3 wt % monoethanolamine, 0.166 wt % tetramethylammonium hydroxide, and 0.005 wt % 1,3,5-benzenetricarboxylic acid (trimesic acid), balance water

Composition CF: 0.3 wt % monoethanolamine, 0.166 wt % tetramethylammonium hydroxide, and 0.006 wt % 1,2,4,5-benzenetetracarboxylic acid (pyromellitic acid), balance water

Composition CG: 0.3 wt % monoethanolamine, 0.166 wt % tetramethylammonium hydroxide, 0.005 wt % 1,2,4-benzenetricarboxylic acid (trimellitic acid), balance water

Composition CH: 0.3 wt % monoethanolamine, 0.166 wt % tetramethylammonium hydroxide, 0.004 wt % 1,2-benzenedicarboxylic acid (phthalic acid), balance water

Composition CI: 0.3 wt % monoethanolamine, 0.166 wt % tetramethylammonium hydroxide, 0.004 wt % 1,3-benzenedicarboxylic acid (isophthalic acid), balance water

Composition CJ: 0.3 wt % monoethanolamine, 0.166 wt % tetramethylammonium hydroxide, 0.004 wt % 1,4-benzenedicarboxylic acid (terephthalic acid), balance water

Composition CK: 0.003% ammonium benzoate, 0.166% tetramethylammonium hydroxide, balance water

Composition CL: 0.003% ammonium benzoate, 0.3% monoethanolamine, balance water

Composition CM: 0.004% phthalic acid, 0.166% tetramethylammonium hydroxide, balance water

Composition CN: 0.004% phthalic acid, 0.3% monoethanolamine, balance water

Composition CO: 9% monoethanolamine, 5% tetramethyl ammonium hydroxide, 3.5% ascorbic acid, balance water

## EXAMPLE 1

PCMP Cleaning Compositions were employed for post CMP cleaning of PCMP 854 wafers (wafers fabricated with the Sematech 854 wafer pattern). The wafers had dried slurry and other PCMP residues on their surface. The wafer in each instance was cleaned on a spin/spray tool with solutions diluted 30:1 (1 part of the composition and 30 parts deionized water as diluent) for 1 minute at 22°C., 100 rpm with a 30 second DI water rinse and spin dry. Pre- and post-cleaning analysis was carried out using a Nanoscope IIIa atomic force microscope.

## 12

The cleaning efficacy was rated by the reduction of objects on the substrate. The particles on the sample substrates were registered as a range of pixels from 231-235 intensity. A Sigma Scan Pro histogram was applied to filter these pixels and count the number of particles. The particle reduction was calculated as:

$$\text{Cleaning Efficacy} = \frac{(\text{Number of PreClean Objects} - \text{Number of Post Clean Objects})}{(\text{Number of PreClean Objects})} \times 100$$

Table 1 below contains the PCMP cleaning data for the foregoing tests, as performed with various complexing agents of the invention, in various compositions as identified hereinabove.

TABLE 1

|    | Cleaning Data      |                   |
|----|--------------------|-------------------|
|    | Formulation (30:1) | Cleaning Efficacy |
| 25 | A                  | ○                 |
|    | B                  | ○                 |
|    | C                  | ○                 |
|    | D                  | ○                 |
|    | E                  | ○                 |
|    | F                  | ○                 |
|    | G                  | ○                 |
|    | H                  | ○                 |
|    | I                  | ○                 |
|    | J                  | ○                 |
|    | K                  | X                 |
|    | L                  | ○                 |
|    | M                  | X                 |
|    | N                  | ○                 |
|    | O                  | X                 |
|    | Q                  | ○                 |
|    | R                  | ○                 |
|    | S                  | ○                 |
|    | T                  | ○                 |
|    | U                  | ○                 |
|    | V                  | ○                 |
|    | W                  | ○                 |
|    | X                  | ○                 |
|    | Y                  | ○                 |
|    | Z                  | ○                 |
|    | AA                 | ○                 |
|    | AB                 | ○                 |
|    | AC                 | ○                 |
|    | AD                 | ○                 |
|    | AE                 | ○                 |
|    | AF                 | ○                 |
|    | AG                 | ○                 |
|    | AH                 | X                 |
|    | AI                 | ○                 |
|    | AJ                 | ○                 |
|    | AK                 | ○                 |
|    | AM                 | ○                 |
|    | AN                 | ○                 |
|    | AO                 | ○                 |
|    | AP                 | ○                 |
|    | AQ                 | ○                 |
|    | AR                 | ○                 |
|    | AS                 | ○                 |
|    | AT                 | ○                 |
| 55 | AU                 | ○                 |

○ = Good Cleaning, cleaning efficacy is greater than 75.

X = Poor Cleaning, cleaning efficacy is less than 75.

The data show that not all complexing agents will provide effective cleaning of the CMP residue from the substrate in the amine/quaternary ammonium hydroxide formulation. Compositions containing cysteine (K), ethylene diamine (M),

glucarate (O), and mucic acid (AH) had poor cleaning efficacy. The data shows that formulations utilizing the complexing agents of the invention cleaned the CMP residues. Examples 2, 13, and 14 will show that while some complexing agents such as citric acid (I), cyanuric acid (J), and tartaric acid (AR) acid have good cleaning efficacy, they are not preferred complexing agents.

## EXAMPLE 2

Surface Preparation for Cobalt Plating Compositions in accordance with the invention were employed for surface preparation of semiconductor wafers, viz., Cu/TEOS 854 wafers (TEOS=tetraethylorthosilicate), for subsequent cobalt plating. The compositions were diluted 40:1 (1 part of the composition and 40 parts deionized water as diluent) and applied to the wafers by static immersion for 30 seconds at 22° C. with a DI water rinse prior to cobalt plating. Analysis was carried out using a JEOL scanning electron microscope (SEM).

A first set of compositions was evaluated, each containing 0.5 wt % tetramethylammonium hydroxide, 1 wt % monoethanolamine, 21 wt %, triethanolamine, 1.5-2.0 wt % complexing agent and balance DI water, against a corresponding control composition containing no complexing agent (composition AV). The complexing agents evaluated in this test were lactic acid (composition AW), oxalic acid (composition AX), and citric acid (composition AY). The control composition contained 0.5 wt % tetramethylammonium hydroxide, 1 wt % monoethanolamine, 21 wt %, triethanolamine and balance DI water.

A second set of compositions was also evaluated, each containing 0.5 wt % TMAH, 0.9 wt % aminoethoxyethanol, 18.7 wt %, dimethylaminoethoxyethanol, 1.5-2.0 wt % complexing agent and balance DI water. The complexing agents evaluated in this test were lactic acid (composition AZ), oxalic acid (composition BA), and citric acid (composition BB).

Selectivity data are shown in Tables 2 and 3, and cobalt deposition quality is shown in the photomicrographs of the cobalt-plated semiconductor device structure in FIGS. 1-7, with the correspondence between the compositions containing the various complexing agents and the photomicrographs of FIGS. 1-7 being set out in Tables 2 and 3.

TABLE 2

| Plating Data for TMAH/MEA/TEA compositions |                        |             |
|--------------------------------------------|------------------------|-------------|
| Formulation (40:1)                         | Selectivity of Plating | FIG. Number |
| AV                                         | Poor                   | 1           |
| AW                                         | Good                   | 2           |
| AX                                         | Good                   | 3           |
| AY                                         | Poor                   | 4           |

TABLE 3

| Plating Data for TMAH/aminoethoxyethanol/dimethylaminoethoxyethanol compositions |                        |             |
|----------------------------------------------------------------------------------|------------------------|-------------|
| Complexing Agent                                                                 | Selectivity of Plating | FIG. Number |
| AZ                                                                               | Good                   | 5           |
| BA                                                                               | Good                   | 6           |
| BB                                                                               | Poor                   | 7           |

The data showed that the plating selectivity for cobalt plating in the respective compositions was good for the compositions containing lactic acid as the complexing agent (compositions AW and AZ) and for the compositions containing oxalic acid as the complexing agent (compositions AX and BA). The micrographs showed significantly improved plating with the compositions utilizing the complexing agents of the invention (FIGS. 2, 3, 5 and 6), as compared to the composition containing no complexing agent (composition AV; FIG. 1) and as compared to the compositions containing citric acid (compositions AY and BB; FIGS. 4 and 7, respectively).

## EXAMPLE 3

15 Copper Attack of 0.18  $\mu$ m Lines on a Device Test Pattern The compositions as described above were tested for copper attack on 854 patterned Cu/TEOS wafers (TEOS=tetraethylorthosilicate). Wafer sections were dipped into solutions diluted 40:1 (1 part of the composition and 40 parts deionized water as diluent), at 22° C. for 5 minutes. The 20 0.1  $\mu$ m lines were analyzed for copper etching by AFM to determine changes in line height and etch rate was measured, in Angstroms per minute. The data are set out in Table 4 25 below.

TABLE 4

| Copper Attack on 0.18 $\mu$ m Lines, as Determined by Change in Line Height, in Angstroms (A), and Measured Etch Rate (ER), in Angstroms Per Minute (A/min) |                       |            |
|-------------------------------------------------------------------------------------------------------------------------------------------------------------|-----------------------|------------|
| Formulation (40:1)                                                                                                                                          | Delta Line Height (A) | ER (A/min) |
| AA                                                                                                                                                          | 13                    | 2.7        |
| BC                                                                                                                                                          | 4                     | 0.9        |
| BD                                                                                                                                                          | 9                     | 1.8        |
| BE                                                                                                                                                          | 3.9                   | 0.8        |
| BF                                                                                                                                                          | 2.9                   | 0.6        |
| BG                                                                                                                                                          | 7.9                   | 1.6        |
| BH                                                                                                                                                          | 8.1                   | 1.6        |
| BI                                                                                                                                                          | 6.2                   | 1.2        |
| BJ                                                                                                                                                          | 11.8                  | 2.4        |
| BK                                                                                                                                                          | 9.4                   | 1.9        |
| BL                                                                                                                                                          | 12.5                  | 2.5        |
| BM                                                                                                                                                          | 6.4                   | 1.3        |
| BN                                                                                                                                                          | 3.0                   | 0.6        |
| BO                                                                                                                                                          | 2.1                   | 0.4        |
| BP                                                                                                                                                          | 7.7                   | 1.5        |
| BQ                                                                                                                                                          | 3.0                   | 0.6        |
| AZ                                                                                                                                                          | 3.9                   | 0.8        |
| BR                                                                                                                                                          | 3.5                   | 0.7        |
| BA                                                                                                                                                          | 2.5                   | 0.5        |
| AW                                                                                                                                                          | 3.3                   | 0.7        |
| BS                                                                                                                                                          | 0                     | 0          |
| AX                                                                                                                                                          | 1.2                   | 0.2        |

55 The data in Table 4 show low levels of attack on the 0.18  $\mu$ m copper lines, with etch rates being less than 3 Angstroms/minute.

## EXAMPLE 4

PCMP Cleaning The compositions identified in Table 5 60 below were diluted 40:1 (1 part of the composition and 40 parts deionized water as diluent) and employed for post CMP cleaning of PCMP 854 wafers. The wafers had dried slurry and other PCMP residues on their surface. The wafer in each instance was cleaned on a spin/spray tool for 1 minute at 22° C., 100 rpm with a 30 second DI water rinse and spin dry. Pre- 65 and post-cleaning analysis was carried out using a Nanoscope IIIa atomic force microscope.

## 15

The cleaning efficacy was rated by the reduction of objects on the substrate. The particles on the sample substrates were registered as a range of pixels from 231-235 intensity. A Sigma Scan Pro's histogram was applied to filter these pixels and count the number of particles. The cleaning efficacy was calculated as:

$$\text{Cleaning Efficacy} = \frac{(\text{Number of PreClean Objects} - \text{Number of Post Clean Objects})}{(\text{Number of PreClean Objects})} \times 100$$

The results of such cleaning test are set out in Table 5 below.

TABLE 5

| Cleaning Data for PCMP Cleaning Compositions |                   |
|----------------------------------------------|-------------------|
| Formulation (40:1)                           | Cleaning Efficacy |
| BC                                           | ○                 |
| BE                                           | ○                 |
| BF                                           | ○                 |
| BN                                           | ○                 |
| BO                                           | ○                 |
| BD                                           | ○                 |
| BG                                           | ○                 |
| BH                                           | ○                 |
| BI                                           | ○                 |
| BK                                           | ○                 |
| BM                                           | ○                 |

○ = Good Cleaning, cleaning efficacy is greater than 75.

X = Poor Cleaning, cleaning efficacy is less than 75.

The data show that these compositions provided effective cleaning of the CMP residue from the substrate.

## EXAMPLE 5

PCMP Cleaning Compositions in accordance with the invention were employed for post CMP cleaning of PCMP 854 wafers. The wafers had dried slurry and other PCMP residues on their surface. The wafer in each instance was cleaned on a spin/spray tool with solutions for 1 minute at 22° C., 100 rpm with a 30 second DI water rinse and spin dry. Pre- and post-cleaning analysis was carried out using a JOEL SEM.

The cleaning efficacy was rated by the reduction of objects on the substrate. The particles on the sample substrates were registered as a range of pixels from 231-235 intensity. A Sigma Scan Pro's histogram was applied to filter these pixels and count the number of particles. The cleaning efficacy was calculated as:

$$\text{Cleaning Efficacy} = \frac{(\text{Number of PreClean Objects} - \text{Number of Post Clean Objects})}{(\text{Number of PreClean Objects})} \times 100$$

The results of such cleaning test are set out in Table 6 below.

## 16

TABLE 6

| Comparative Cleaning Performance |             |                   |
|----------------------------------|-------------|-------------------|
| 5                                | Formulation | Cleaning Efficacy |
| 10                               | CB          | ○                 |
|                                  | CC          | ○                 |
|                                  | CD          | ○                 |
|                                  | CE          | ○                 |
|                                  | CF          | ○                 |
|                                  | CB          | ○                 |
|                                  | CH          | ○                 |
|                                  | CI          | ○                 |
|                                  | CJ          | ○                 |

○ = Good Cleaning, cleaning efficacy is greater than 75.

X = Poor Cleaning, cleaning efficacy is less than 75.

The foregoing data show that the compositions yielded excellent cleaning efficiency.

## EXAMPLE 6

Copper Roughening Cleaning solutions CA-CJ were evaluated for their effect on copper corrosion.

Copper wafer sections were obtained from a polished copper wafer, and the sections were treated according to the cleaning test procedure of Example 5. After treatment, the copper wafer sections were subjected to AFM examination to determine the nature and extent of surface roughening. The results are set out in Table 7 below.

TABLE 7

| Cu Roughening Data |             |                |
|--------------------|-------------|----------------|
|                    | Formulation | Roughness (nm) |
| 35                 | Untreated   | 0.7            |
|                    | CB          | 0.7            |
|                    | CC          | 0.7            |
|                    | CD          | 0.7            |
|                    | CE          | 0.7            |
|                    | CF          | 0.7            |
|                    | CG          | 0.7            |
|                    | CH          | 0.7            |
|                    | CI          | 0.7            |
|                    | CJ          | 0.7            |

The foregoing data show that the compositions have low roughening. They did not change the roughness of the copper samples.

## EXAMPLE 7

Composition Component Synergy Cleaning compositions CK-CN were evaluated to determine the effect of quaternary ammonium hydroxide and amine on cleaning in the compositions of the invention.

The cleaning compositions were employed for post CMP cleaning of PCMP 854 wafers (wafers fabricated with the Sematech 854 wafer pattern). The wafers had dried slurry and other PCMP residues on their surface. The wafer in each instance was cleaned on a spin/spray tool with dilute solutions for 1 minute at 22° C., 100 rpm with a 30 second DI water rinse and spin dry. Pre- and post-analysis was performed using a Nanoscope IIIa atomic force microscope.

The cleaning efficacy was rated by the reduction of objects on the substrate. The particles on the sample substrates were registered as a range of pixels from 231-235 intensity. A Sigma Scan Pro histogram was applied to filter these pixels and count the number of particles. The cleaning efficacy was calculated as:

$$\text{Cleaning Efficacy} = \frac{(\text{Number of PreClean Objects} - \text{Number of Post Clean Objects})}{(\text{Number of PreClean Objects})} \times 100$$

The results of such cleaning test are set out in Table 8.

TABLE 8

| Comparative Cleaning Performance |                   |
|----------------------------------|-------------------|
| Formulation                      | Cleaning Efficacy |
| CK                               | X                 |
| CL                               | X                 |
| CM                               | X                 |
| CN                               | X                 |

O = Good Cleaning, cleaning efficacy is greater than 75.

X = Poor Cleaning, cleaning efficacy is less than 75.

The foregoing data shows the synergy between the components. When a major component such as amine or quaternary ammonium hydroxide is not present in the formulation, the cleaning fails.

## EXAMPLE 8

Copper Etch Rate by Electrochemistry Cleaning solutions were prepared, and evaluated for copper etch rate performance.

Corrosion (etch) rates were determined from Tafel plots generated by potentiodynamic scans from -150 to +150 mV versus open circuit potential at a scan rate of 0.25 mV/sec. The working electrode was a 5 mm diameter copper rod (99.999% pure, Alfa Inorganics) potted in epoxy inside of a Teflon® polytetrafluoroethylene tube. The working electrode was cleaned prior to each use. The counter electrode was a 1 mm platinum wire (Alfa Inorganics) and the reference electrode was a silver-silver chloride (saturated KCl) electrode (Princeton Applied Research Corp.). The potentiostat was a Princeton Applied Research Model 2263. The copper electrode was first oxidized at +0.700V for 5 minutes and then allowed to go to the open circuit potential for 1 hour. The potentiodynamic scan was then performed, and the calculations were done using software provided by Princeton Applied Research Corporation, to determine the corrosion rate.

The results are shown in Table 9 below.

TABLE 9

| Copper Etch Rate Results |                               |
|--------------------------|-------------------------------|
| Formulation              | Copper Corrosion Rate (Å/min) |
| B                        | 3.1                           |
| M                        | 11.5                          |
| U                        | 3.3                           |
| V                        | 3.3                           |
| Y                        | 2.6                           |
| AA                       | 3.9                           |
| AE                       | 3.5                           |
| AG                       | 0.01                          |
| AI                       | 3.4                           |
| AN                       | 2.8                           |
| BC                       | 0.6                           |
| CB                       | 3.2                           |
| CC                       | 3.5                           |
| CD                       | 1.8                           |

TABLE 9-continued

| 5  | Formulation | Copper Etch Rate Results      |  |
|----|-------------|-------------------------------|--|
|    |             | Copper Corrosion Rate (Å/min) |  |
| 10 | CE          | 6.1                           |  |
|    | CF          | 2.2                           |  |
|    | CG          | 2.9                           |  |
|    | CH          | 2.2                           |  |
|    | CI          | 5.8                           |  |
|    | CJ          | 2.3                           |  |

The data in Table 9 shows that the compositions in accordance with the invention have low corrosion rates, less than 7 Å/min. 15 Composition M containing ethylene diamine as a complexing agent has a very high corrosion rate, greater than 7 Å/min.

## EXAMPLE 9

20 Benzotriazole (BTA) Removal Cleaning compositions were used to clean a copper seed wafer contaminated using a 10 ppm BTA solution during 1 hour with static immersion, followed by deionized (DI) water rinsing then blown dry with nitrogen. The samples were cleaned on a spin/spray tool for 1 minute at 22° C., 100 rpm with a 30 second DI water rinse and spin dry. Analysis was done using XPS at an angle of 15°. The compositions were used at a dilution of 30:1 (1 part of the composition and 30 parts deionized water as diluent). Data are shown in Table 10 below.

TABLE 10

| BTA Removal by TMAH/MEA Compositions |                      |           |        |          |                 |                           |
|--------------------------------------|----------------------|-----------|--------|----------|-----------------|---------------------------|
| Pre-treatment                        | Cleaning Formulation | XPS Angle | Copper | Nitrogen | Nitrogen/Copper | % BTA Removed by Cleaning |
| None                                 | None                 | 15        | 94.1   | 5.9      | 0.06            | Not applicable            |
| BTA                                  | None                 | 15        | 28.0   | 72.0     | 2.57            | Not applicable            |
| 40                                   | U                    | 15        | 95.2   | 4.8      | 0.05            | 100                       |
| BTA                                  | AA                   | 15        | 95.7   | 4.3      | 0.05            | 100                       |
| BTA                                  | AQ                   | 15        | 94.0   | 6.0      | 0.06            | 100                       |

45 The data in Table 10 shows that the formulations remove the BTA contamination. The nitrogen/copper ratio is equal to the uncontaminated copper sample after treatment with the formulations. There is effectively 0% BTA left on the samples after cleaning.

## EXAMPLE 10

Post Etch Residue Removal Compositions were used to clean post etch wafers contaminated with residue in the vias. The wafers were cleaned on a spin/spray tool for 45 seconds at 22° C., 100 rpm with a 15 second DI water rinse and spin dry. Analysis was conducted using a JEOL SEM.

The results are set out in Table 11 below.

TABLE 11

| Post Etch Residue Removal by Compositions in a Spin/Spray Application |                      |         |
|-----------------------------------------------------------------------|----------------------|---------|
|                                                                       | Cleaning Formulation | Residue |
| 60                                                                    | Untreated            | Present |
| 65                                                                    | U                    | Removed |
|                                                                       | AA                   | Removed |

TABLE 11-continued

| Post Etch Residue Removal by Compositions in a Spin/Spray Application |         |
|-----------------------------------------------------------------------|---------|
| Cleaning Formulation                                                  | Residue |
| AQ                                                                    | Removed |
| CO                                                                    | Present |

The ascorbic acid-containing composition CO was not as efficient at removing the post etch residue as the glycine-containing composition U, the lactic acid-containing composition AA or the succinic acid-containing composition AQ.

## EXAMPLE 11

Post Etch Residue Removal Compositions were used to clean post etch wafers contaminated with residue in the vias. The wafers were cleaned by static immersion for 2 minutes at 22° C., with a 15 second DI water rinse and N<sub>2</sub> dry. Analysis was done using a JEOL SEM.

The results are set out in Table 12 below.

TABLE 12

| Post Etch Residue Removal by Compositions in an Immersion Application |         |
|-----------------------------------------------------------------------|---------|
| Cleaning Formulation                                                  | Residue |
| Untreated                                                             | Present |
| U                                                                     | Removed |
| AA                                                                    | Removed |
| AQ                                                                    | Removed |

Similar to Example 10, the glycine-containing composition U, the lactic acid-containing composition AA and the succinic acid-containing composition AQ were efficient at removing the post etch residue in an immersion treatment.

## EXAMPLE 12

**Copper Etching** The same compositions as tested in Example 11, as well as a corresponding TMAH/MEA composition containing gallic acid as the complexing agent in accordance with the disclosure of U.S. Pat. No. 6,194,366, were used to clean unpolished PVD copper wafers. About 1000 Angstroms of copper had been deposited on these wafers by physical vapor deposition.

The wafers were cleaned by static immersion at increments of 1, 2, 3 and 4 minutes at 22° C., followed by a 15 second DI water rinse and N<sub>2</sub> dry. Thickness measurements were made with a CD ResMap 4 point probe.

The etch rates of copper measured for the compositions of Example 11 were less than the etch rate measured for the gallic acid-containing composition of U.S. Pat. No. 6,194,366. FIG. 8 is a graph of etch rates, in Angstroms per minute, for the respective TMAH/MEA compositions containing the different complexing agents (gallic acid (P), lactic acid (AA), glycine (U), succinic acid (AQ), 2-mercaptopbenzimidazole (BU), and lactic acid with 2-mercaptopbenzimidazole (BT)), on the copper substrate.

## EXAMPLE 13

**Copper Roughening Compositions** in accordance with the invention were employed to clean polished copper wafers. The wafer in each instance was cleaned on a spin/spray tool for 1 minute at 22° C., 100 rpm with a 30 second DI water

rinse and spin dry. Analysis was carried out using a Nanoscope IIIa atomic force microscope.

FIG. 9 is a graph of surface roughness, in nm, for various TMAH/MEA compositions described previously, showing the relative magnitudes of the roughness associated with varying complexing agents, compared to an untreated copper surface having a roughness of 1.4 nm. Low roughness is less than 1.8 nm of roughness. High roughness is greater than 1.8 nm or roughness.

The data in FIG. 9 show that formulations in accordance to the invention have low roughness. Complexing agents such as citric acid (I) and cyanuric acid (J) previously showed good cleaning efficacy in Example 1, but these formulations have unacceptable amounts of roughness. Complexing agents such as cysteine (K) and ethylene diamine (M) previously showed poor cleaning efficacy in Example 1 and have high roughness. This shows that etching the surface is not a sufficient method for removing CMP residue.

## EXAMPLE 14

**Copper Roughening Compositions** in accordance with the invention were employed to clean polished copper wafers. The wafer in each instance was cleaned on a spin/spray tool for 1 minute at 22° C., 100 rpm with a 30 second DI water rinse and spin dry. Analysis was carried out using a Nanoscope IIIa atomic force microscope.

FIG. 10 is a graph of surface roughness, in nm, for various TMAH/MEA compositions described previously, showing the relative magnitudes of the roughness associated with varying complexing agents, compared to an untreated copper surface having a roughness of 1.4 nm.

The data in FIG. 10 show that formulations in accordance to the invention have low roughness. Complexing agent tartaric acid (AR) previously showed good cleaning efficacy in Example 1, but this formulation produces unacceptable amounts of roughness.

## EXAMPLE 15

FIGS. 11-20 are photomicrographs of post-etch wafers, at respective magnifications of 40,000 $\times$  and 80,000 $\times$ . FIGS. 11 and 12 show the wafer as untreated. In all other cases, the wafers were cleaned on a spin/spray tool for 45 seconds at 22° C., 100 rpm with a 15 second DI water rinse and spin dry. FIGS. 13 and 14 show the wafer after spin/spray cleaning with the lactic acid-containing TMAH/MEA composition AA. FIGS. 15 and 16 show the wafer after spin/spray cleaning with the glycine-containing TMAH/MEA composition U. FIGS. 17 and 18 show the wafer after spin/spray cleaning with the succinic acid-containing TMAH/MEA composition AQ. FIGS. 19 and 20 show the wafer after spin/spray cleaning with the ascorbic acid-containing TMAH/MEA composition CO.

More specifically, FIG. 11 is a photomicrograph at magnification of 40,000 $\times$  of a post-etch wafer showing residue in vias therein.

FIG. 12 is a photomicrograph of the post-etch wafer of FIG. 11, at a magnification of 80,000 $\times$ , showing the residue in the vias, in greater detail.

FIG. 13 is a photomicrograph at magnification of 40,000 $\times$  of the post-etch wafer shown in FIG. 11, after cleaning by spin/spray with the TMAH/MEA/lactic acid aqueous cleaning composition AA. The post etch residue in the via was removed by the cleaning composition.

## 21

FIG. 14 is a photomicrograph of the post-etch wafer of FIG. 13, at a magnification of 80,000 $\times$ , showing the removal of the post-etch residue in the via, in greater detail.

FIG. 15 is a photomicrograph at magnification of 40,000 $\times$  of the post-etch wafer shown in FIG. 1, after cleaning by spin/spray with the TMAH/MEA/glycine aqueous cleaning composition U. The post etch residue in the via was removed by the cleaning composition.

FIG. 16 is a photomicrograph of the post-etch wafer of FIG. 15, at a magnification of 80,000 $\times$ , showing the removal of the post-etch residue in the via, in greater detail.

FIG. 17 is a photomicrograph at magnification of 40,000 $\times$  of the post-etch wafer shown in FIG. 11, after cleaning by spin/spray with the TMAH/MEA/succinic acid aqueous cleaning composition AQ. The post etch residue in the via was removed by the cleaning composition.

FIG. 18 is a photomicrograph of the post-etch wafer of FIG. 17, at a magnification of 80,000 $\times$ , showing the removal of the post-etch residue in the via, in greater detail.

FIG. 19 is a photomicrograph at magnification of 40,000 $\times$  of the post-etch wafer shown in FIG. 11, after cleaning by spin/spray with the TMAH/MEA/ascorbic acid aqueous cleaning composition CO. The post etch residue still remained in the via after treatment by the cleaning composition.

FIG. 20 is a photomicrograph of the post-etch wafer of FIG. 19, at a magnification of 80,000 $\times$ , showing the post-etch residue remaining in the via, in greater detail.

## EXAMPLE 16

FIGS. 21-25 are photomicrographs of post-etch wafers, at respective magnifications of 40,000 $\times$  and 80,000 $\times$ , after cleaning of the wafer by static immersion for 2 minutes at 22° C., with a 15 second DI water rinse and N<sub>2</sub> dry. FIGS. 21 and 22 show the wafer after immersion cleaning with the lactic acid-containing TMAH/MEA composition AA. FIG. 23 shows the wafer after immersion cleaning with the glycine-containing TMAH/MEA composition U. FIGS. 24 and 25 show the wafer after immersion cleaning with the succinic acid-containing TMAH/MEA composition AQ.

More specifically, FIG. 21 is a photomicrograph at magnification of 40,000 $\times$  of the post-etch wafer shown in FIG. 11, after immersion cleaning with the TMAH/MEA/lactic acid aqueous cleaning composition AA. The post etch residue in the via was removed by the cleaning composition.

FIG. 22 is a photomicrograph of the post-etch wafer of FIG. 21, at a magnification of 80,000 $\times$ , showing the removal of the post-etch residue in the via, in greater detail.

FIG. 23 is a photomicrograph at magnification of 40,000 $\times$  of the post-etch wafer shown in FIG. 11, after immersion cleaning with the TMAH/MEA/glycine aqueous cleaning composition U. The post etch residue in the via was removed by the cleaning composition.

FIG. 24 is a photomicrograph at magnification of 40,000 $\times$  of the post-etch wafer shown in FIG. 11, after immersion cleaning with the TMAH/MEA/succinic acid aqueous cleaning composition AQ. The post etch residue in the via was removed by the cleaning composition.

FIG. 25 is a photomicrograph of the post-etch wafer of FIG. 24, at a magnification of 80,000 $\times$ , showing the removal of the post-etch residue in the via, in greater detail.

While the invention has been described herein in reference to specific aspects, features and illustrative embodiments of the invention, it will be appreciated that the utility of the invention is not thus limited, but rather extends to and encompasses numerous other variations, modifications and

## 22

alternative embodiments, as will suggest themselves to those of ordinary skill in the field of the present invention, based on the disclosure herein. Correspondingly, the invention as hereinafter claimed is intended to be broadly construed and interpreted, as including all such variations, modifications and alternative embodiments, within its spirit and scope.

What is claimed is:

1. A composition comprising (i) alkanolamine, (ii) quaternary ammonium hydroxide and (iii) a complexing agent, wherein the complexing agent includes at least one component selected from the group consisting of glyoxylic acid, 2-mercaptopbenzimidazole, proline, and derivatives of the foregoing amino acids, with the provision that the complexing agent does not include citric acid, and wherein the composition has a pH greater than 9.
2. The composition of claim 1, wherein components (i), (ii), and (iii) are in effective relative proportions to one another for surface preparation and/or cleaning of a semiconductor substrate.
3. The composition of claim 1, including about 0.001 to about 90 wt. % alkanolamine, about 0.00001 to about 40 wt. % quaternary ammonium hydroxide, and about 0.00001 to about 20 wt. % complexing agent, based on total weight of the composition.
4. The composition of claim 1, wherein the alkanolamine is present in an amount of from about 0.001 wt. % to about 90 wt. %, based on the weight of the composition.
5. The composition of claim 1, wherein the quaternary ammonium hydroxide is present in an amount of from about 0.005 wt. % to about 40 wt. % based on the weight of the composition.
6. The composition of claim 1, wherein the complexing agent is present in an amount of from about 0.001 wt. % to about 20 wt. %, based on the weight of the composition.
7. The composition of claim 1, further comprising water.
8. The composition of claim 7, containing less than 20 wt. % water, based on total weight of the composition.
9. The composition of claim 7, wherein water is present in an amount of from about 95 wt. % to about 99.999 wt. %, based on the weight of the composition.
10. The composition of claim 1, wherein the alkanolamine includes at least one species selected from the group consisting of aminoethylethanolamine, N-methylaminoethanol, aminoethoxyethanol, dimethylaminoethoxyethanol, diethanolamine, N-methyldiethanolamine, monoethanolamine, triethanolamine, and C<sub>1</sub>-C<sub>8</sub> alkanolamines.
11. The composition of claim 1, wherein the quaternary ammonium hydroxide is selected from the group consisting of choline, tetrabutylammonium hydroxide, tetraethylammonium hydroxide, tetramethylammonium hydroxide, tetrapropylammoniumhydroxide, and combinations thereof.
12. The composition of claim 1, having a pH greater than 10.
13. The composition of claim 1, wherein components (i), (ii), and (iii) are in relative proportions rendering the composition non-darkening and degradation-resistant in exposure to oxygen.
14. The composition of claim 1, wherein the complexing agent further includes at least one species selected from the group consisting of lactic acid, glycine, succinic acid and oxalic acid.
15. A method of processing a semiconductor substrate to remove undesired material therefrom or to prepare a surface of said semiconductor substrate for subsequent treatment, said method comprising contacting the semiconductor substrate with an effective amount of a composition comprising (i) alkanolamine, (ii) quaternary ammonium hydroxide and

(iii) a complexing agent, wherein the complexing agent includes at least one component selected from the group consisting of glyoxylic acid, 2-mercaptopbenzimidazole, proline, and derivatives of the foregoing amino acids, with the provision that the complexing agent does not include citric acid, and wherein the composition has a pH greater than 9.

16. The method of claim 15, comprising processing the semiconductor substrate to remove etch residue or chemical mechanical polishing residue therefrom.

17. The method of claim 15, comprising processing the semiconductor substrate to remove BTA therefrom.

18. The method of claim 15, comprising processing the semiconductor substrate to prepare it for subsequent deposition of material thereon.

19. The method of claim 18, wherein said deposition of material comprises cobalt plating.

20. The method of claim 15, wherein components (i), (ii), and (iii) are in effective relative proportions to one another for surface preparations and/or cleaning of a semiconductor substrate.

21. The method of claim 15, wherein the composition includes about 0.001 to about 90 wt. % alkanolamine, about 0.00001 to about 40 wt. % quaternary ammonium hydroxide, and about 0.00001 to about 20 wt. % complexing agent, based on total weight of the composition.

22. The method of claim 15, wherein the composition includes alkanolamine in an amount of from about 0.001 wt. % to about 90 wt. %, based on the weight of the composition.

23. The method of claim 15, wherein the composition includes quaternary ammonium hydroxide in an amount of from about 0.005 wt. % to about 40 wt. %, based on the weight of the composition.

24. The method of claim 15, wherein the composition includes complexing agent in an amount of from about 0.001 wt. % to about 20 wt. % based on the weight of the composition.

25. The method of claim 15, wherein the composition includes water.

26. The method of claim 25, wherein the composition includes less than 20 wt. % water, based on total weight of the composition.

27. The method of claim 25, wherein the composition includes water in an amount of from about 95 wt. % to about 99.999 wt. %, based on the weight of the composition.

28. The method of claim 15, wherein the composition comprises alkanolamine including at least one species selected from the group consisting of aminoethylethanolamine, N-methylaminoethanol, aminoethoxyethanol, dimethylaminoethoxyethanol, diethanolamine, N-methyldiethanolamine, monoethanolamine, triethanolamine, and C<sub>1</sub>-C<sub>8</sub> alkanolamines.

29. The method of claim 15, wherein the composition comprises quaternary ammonium hydroxide selected from the group consisting of choline, tetrabutylammoniumhydroxide, tetraethylammonium hydroxide, tetramethylammonium hydroxide, tetrapropylammoniumhydroxide, and combinations thereof.

30. The method of claim 15, wherein the pH is greater than 10.

31. The method of claim 15, wherein the composition comprises components (i), (ii), and (iii) in relative proportions rendering the composition non-darkening and degradation-resistant in exposure to oxygen.

32. The method of claim 15, wherein the composition further comprises complexing agent including at least one species selected from the group consisting of lactic acid, glycine, succinic acid and oxalic acid.

33. The composition of claim 1, comprising monoethanolamine, tetramethylammonium hydroxide, 2-mercaptopbenzimidazole and water.

34. The composition of claim 1, comprising monoethanolamine, tetramethylammonium hydroxide, 2-mercaptopbenzimidazole, lactic acid, and water.

35. A composition comprising (i) alkanolamine, (ii) quaternary ammonium hydroxide, (iii) a complexing agent and (iv) water, wherein the complexing agent includes at least one component selected from the group consisting of 2-mercaptopbenzimidazole, proline, and derivatives of the foregoing amino acids, with the provision that the complexing agent does not include citric acid, and wherein the composition has a pH greater than 9.

\* \* \* \* \*

UNITED STATES PATENT AND TRADEMARK OFFICE  
**CERTIFICATE OF CORRECTION**

PATENT NO. : 7,923,423 B2  
APPLICATION NO. : 11/046262  
DATED : April 12, 2011  
INVENTOR(S) : Walker et al.

Page 1 of 1

It is certified that error appears in the above-identified patent and that said Letters Patent is hereby corrected as shown below:

Title Pg, Item (75) Inventors: please add "Kevin P. Yanders, Germansville, PA (US)" and  
"Darryl W. Peters, Stewartsville, NJ (US)"

Signed and Sealed this  
Thirty-first Day of May, 2011



David J. Kappos  
*Director of the United States Patent and Trademark Office*